

## UNITED STATES PATENT OFFICE

1,976,218

TREATMENT OF MATERIAL CONTAINING  
ORGANIC ESTERS OF CELLULOSE

Camille Dreyfus, New York, N. Y., and William Whitehead, Cumberland, Md., assignors to Celanese Corporation of America, a corporation of Delaware

No Drawing. Application September 8, 1928,  
Serial No. 304,809

8 Claims. (Cl. 28—59)

This invention relates to the treatment of materials such as yarns, filaments, bristles, films, fabrics, etc., made of or containing organic derivatives of cellulose in such a manner as to de-lustre or render the same more opaque without causing the same to crinkle.

An object of our invention is to reduce the lustre or increase the opacity of materials containing organic esters of cellulose in such a manner that they do not crinkle or otherwise become distorted. Other objects of our invention will appear from the following detailed description.

Textile materials such as yarns, fabrics and the like containing organic derivatives of cellulose may be rendered more opaque and their lustre may be reduced by subjecting the same to the action of boiling water or wet steam. However, if the textile material is subjected to such agencies in the ordinary manner they tend to crinkle, warp or otherwise become distorted. We have found, however, that if such materials are subjected to the delustering agency while they are under tension, the tendency to crinkle or warp is reduced or overcome.

In accordance with our invention, we subject the material made of or containing organic esters of cellulose to the action of an agent that tends to reduce the lustre and/or increase the opacity of the organic ester of cellulose material while such material is under a tension or stress.

The material to be treated in accordance with our invention may be filaments or yarns such as are used in making fabric. Moreover the fabric itself may be treated advantageously by our process. An important application of our invention is the treatment of bristles or artificial horse hair such as are used in hair brushes or clothes brushes, since bristles of reduced lustre but which are straight are required for this work. Also films, fibres or other filaments may be treated by our invention if so desired.

The organic ester of cellulose of which the material is composed or which the material contains, may be any suitable one, examples of which are cellulose acetate, cellulose formate, cellulose propionate or cellulose butyrate.

The delustering agency employed may be any suitable one. However, for ease of application we prefer wet steam or boiling water. The boiling water may contain other substances such as soap, salts, acid salts, acids and particularly aliphatic carboxylic acids, such as acetic acid or formic acid which either increase, decrease or have no effect upon the rate of delustering.

The time of treatment of the organic ester of

cellulose material may be varied in accordance with the effect desired. A short treatment merely increases the opacity while longer treatments also affect the optical smoothness of the material and reduce the lustre thereof. Depending upon the time of treatment the lustre may be slightly reduced or the material may be completely delustered. When wet steam is employed it is preferable to first dampen them or wet the material to be treated with water prior to treatment with wet steam in order to promote uniform delustering.

The material undergoing the delustering treatment may be subjected to tension or stress in any suitable manner. In one form of carrying out the process weights may be suspended from the material while it is being subjected to the delustering agency. In another form, the yarns, fabrics, films or bristles to be treated may be wound from reel to reel under tension while being drawn through the delustering agency. The load or tension on the material obviously should not exceed that of the breaking load. By way of example it may be stated that a load of 1 gram for every 50 denier of yarn or bristle, and a corresponding load for film or fabric is quite suitable.

The yarns, bristles, films, etc., may be subjected to the delustering process directly after their formation in a spinning machine or on a film wheel, being passed from the feed rollers or wheels of the forming machine directly through steam chests or boiling baths under tension.

The yarns, fabrics, bristles or films after having been subjected to the process of our invention are relatively opaque and have a reduced lustre ranging from a slight delustering to complete delustering. Because of the tension under which they have been subjected while being treated they are free of crinkling, curling, warping or other distortions.

In order further to illustrate our invention the following specific examples are given without limiting the scope thereof.

## Example I

100

A hank of artificial bristles of 100 denier which bristles consist of an acetone soluble cellulose acetate having an acetyl value of 54.5% is treated. A hank weighing 320 grams is hung in a steam chest, preferably after wetting, but not necessarily so, and is subjected to the action of wet steam at 80° C. for 10 minutes. The hank is suspended on a bar which passes under the upper end thereof. Another bar is suspended from the lower end 110

of the hank and this bar is loaded with a weight of 10 kilograms.

By this process an opaque bristle suitable for hair brushes, etc., with a reduced lustre is obtained which bristle is free of any distortion, crinkling, etc.

*Example II*

The procedure of Example I is repeated substituting, however, a yarn of 150 denier containing 26 individual filaments, which yarn is spun from a similar cellulose acetate.

By this process an opaque yarn of subdued lustre and entirely devoid of crinkling or other distortion is obtained. This yarn is capable of being wound from hank to bobbin, pirn or other package, without the constant catching or breaking that otherwise occurs if the yarn is delustered in the ordinary manner and not under tension.

By repeating this process but increasing the time of steaming to 30 minutes, a yarn is obtained that is smooth and undistorted and has an opaque and matte appearance.

It is to be understood that the foregoing detailed description is given merely by way of illustration and that many variations may be made therein without departing from the spirit of this invention.

Having described our invention what we claim and desire to secure by Letters Patent is:

1. Process of producing at least partially delustered yarns containing organic esters of cellulose which comprises suspending the yarns in hank form, attaching weights to said hanks and subjecting the hanks to the action of a hot aqueous delustering medium while thus tensioned so as to prevent crinkling.

2. Process of producing at least partially delustered yarns containing cellulose acetate which comprises suspending the yarns in hank form, attaching weights to said hanks and subjecting the hanks to the action of a hot aqueous delustering medium while thus tensioned so as to prevent crinkling.

3. Process of producing at least partially delustered textile material containing organic esters of cellulose which comprises wetting the textile

material, suspending the same in hank form, attaching weights to said textile material and subjecting the textile material to the action of a hot aqueous delustering medium while thus tensioned so as to prevent crinkling.

4. Process of producing at least partially delustered textile material containing cellulose acetate which comprises wetting the textile material, suspending the same in hank form, attaching weights to said textile material and subjecting the textile material to the action of a hot aqueous delustering medium while thus tensioned so as to prevent crinkling.

5. Process of producing at least partially delustered yarns containing organic esters of cellulose which comprises wetting the yarns, suspending the same in hank form, attaching weights to said hanks and subjecting the hanks to the action of a hot aqueous delustering medium while thus tensioned so as to prevent crinkling.

6. Process of producing at least partially delustered yarns containing cellulose acetate which comprises wetting the yarns, suspending the same in hank form, attaching weights to said hanks and subjecting the hanks to the action of a hot aqueous delustering medium while thus tensioned so as to prevent crinkling.

7. Process of producing at least partially delustered yarns containing organic esters of cellulose which comprises suspending the yarns in hank form from a rod, passing another rod through the bottom of the hanks, attaching a weight to said lower rod so as to impart tension to the yarns in the hanks and subjecting the hanks to the action of a hot aqueous delustering medium while thus tensioned so as to prevent crinkling.

8. Process of producing at least partially delustered yarns containing cellulose acetate which comprises suspending the yarns in hank form from a rod, passing another rod through the bottom of the hanks, attaching a weight to said lower rod so as to impart tension to the yarns in the hanks and subjecting the hanks to the action of a hot aqueous delustering medium while thus tensioned so as to prevent crinkling.

CAMILLE DREYFUS.  
WILLIAM WHITEHEAD.

50

125

55

130

60

135

65

140

70

145

75

150